

# United States Patent

[19]

Minagawa et al.

[11] 3,996,055

[45] Dec. 7, 1976

[54] **COLOR PHOTOGRAPHIC  
LIGHT-SENSITIVE MATERIAL**

[75] Inventors: **Yoshisato Minagawa; Akio  
Okumura**, both of Minami-ashigara,  
Japan

[73] Assignee: **Fuji Photo Film Co., Ltd.,**  
Minami-ashigara, Japan

[22] Filed: **Dec. 23, 1974**

[21] Appl. No.: **535,752**

[30] **Foreign Application Priority Data**

Dec. 21, 1973 Japan ..... 49-3113

[52] **U.S. Cl.** ..... **96/74; 96/9;**  
96/55; 96/95; 96/100

[51] **Int. Cl.<sup>2</sup>** ..... **G03C 1/76**

[58] **Field of Search** ..... 96/9, 74, 100

[56] **References Cited**

UNITED STATES PATENTS

3,615,602 10/1971 Credner et al. ..... 96/100

|           |        |                    |       |
|-----------|--------|--------------------|-------|
| 3,642,485 | 2/1972 | Oishi et al. ....  | 96/74 |
| 3,658,545 | 4/1972 | Iwama et al. ....  | 96/9  |
| 3,784,383 | 1/1974 | Iwama et al. ....  | 96/9  |
| 3,811,892 | 5/1974 | Kagami et al. .... | 96/9  |

*Primary Examiner*—J. Travis Brown

*Attorney, Agent, or Firm*—Sughrue, Rothwell, Mion,  
Zinn & Macpeak

[57] **ABSTRACT**

A color photographic light-sensitive material, comprising a support having thereon at least one silver halide emulsion and the light sensitive material containing a colored cyan coupler having a main absorption in the blue region of the spectrum and a colored cyan coupler having a main absorption in the green region of the spectrum, and a colorless cyan coupler, each coupler being capable of coupling with an oxidation product of a p-phenylenediamine color-developing agent to form a cyan dye.

**10 Claims, 3 Drawing Figures**

FIG. I



**FIG. 2****FIG. 3**

**FIG.4**



**FIG.5**



## COLOR PHOTOGRAPHIC LIGHT-SENSITIVE MATERIAL

### BACKGROUND OF THE INVENTION

#### 1. Field of the Invention

The present invention relates to a color photographic light-sensitive material, and, more particularly to a silver halide color negative light-sensitive material capable of providing a color print dye image having excellent color reproducibility.

#### 2. Description of the Prior Art

It is well known that, when a silver halide color photographic material is color-developed, a color-forming coupler couples with an oxidation product of an aromatic primary amine developing agent to form a dye image of an indophenol, indamine, azomethine, phenoxazine, phenazine or a like structure. In this system, a color reproduction process based on subtractive color photography is usually employed, and a cyan dye image, a magenta dye image and a yellow dye image, which are in a complementary relationship with the original red, green and blue, respectively, of the object photographed, are formed. Usually, phenolic couplers (i.e., phenols and naphthols) are used for the formation of a cyan-dye image, pyrazolone or cyanoacetyl couplers are used for the formation of a magenta dye image, and acylacetamides or benzoylmethane couplers are used for the formation of a yellow dye image.

The thus formed dye image does not possess theoretically ideal spectral absorption characteristics. For example, a cyan dye image generally has side-absorptions of green light and blue light, although it should only absorb red light. Also, a magenta dye image generally has side-absorptions of blue light and red light, although it should only absorb green light. A yellow dye image has comparatively small side-absorption as compared with the above-described cyan and magenta dye images. Such side-absorptions are not advantageous for the color reproducibility of a light-sensitive material. As a process for removing this defect, a so-called masking process using a colored color-forming coupler has been put into practice in this field (for example, as disclosed in U.S. Pat. No. 2,428,054). Color prints obtained from the masked color negative images have excellent color reproducibility.

According to the masking process, as described in U.S. Pat. No. 2,428,054, etc., it is desirable to use a cyan coupler which is colored so that it has absorption in the blue region and the green region (hereinafter referred to as "colored cyan coupler) in combination with a colorless cyan coupler, in order to remove the above-described cyan dye side-absorptions.

Colored cyan couplers are described in U.S. Pat. Nos. 3,481,741, 3,459,552, 3,583,971, 2,455,169, 3,034,892, etc. However, these colored cyan couplers have the defect that those cyan couplers which have sufficient absorption in the blue region have insufficient absorption in the green region while those which have sufficient absorption in the green region have insufficient absorption in the blue region. Therefore, these colored couplers have insufficient masking properties.

### SUMMARY OF THE INVENTION

Therefore, an object of the present invention is to provide a silver halide color negative photographic light-sensitive material having good color reproducibility.

Another object of the present invention is to provide a process for effecting color correction of a cyan dye through masking using a colored cyan coupler having an unsatisfactory spectral absorption characteristics when the colored cyan coupler is used alone.

These and other objects are attained with both a colored cyan coupler having a main absorption in the blue region and a colored cyan coupler having a main absorption in the green region in combination with a colorless cyan coupler.

The color light-sensitive material of the present invention comprises a support having thereon at least one silver halide photographic emulsion layer containing a color coupler, wherein the silver halide emulsion layer sensitive to red light contains in combination a colored cyan coupler having a main absorption in the blue region of the spectrum, a colored cyan coupler having a main absorption in the green region of the spectrum, and a colorless cyan coupler.

### BRIEF DESCRIPTION OF THE DRAWINGS

FIG. 1 shows the spectral absorption curves of 5 typical compounds of colored cyan couplers having a main absorption in the blue region and colored cyan couplers having a main absorption in the green region measured in an organic solvent (tricresylphosphate), wherein Curves (1), (2), (3), (4) and (5) are the spectral absorption spectra of Compounds (31), (35), (41), (4) and (21), respectively.

FIGS. 2 through 5 illustrate the color-correcting effect of the present invention, wherein Curves R, G and B show the characteristic curves of a cyan color image obtained by red photometry, green photometry and blue photometry, respectively.

### DETAILED DESCRIPTION OF THE INVENTION

The colored cyan couplers of the present invention having a main absorption in the blue region are those couplers which have an absorption peak in the wavelength range of about 390 to 490 nm, and the colored cyan couplers having a main absorption in green region are those couplers which have an absorption peak in the wavelength range of about 490 to 550 nm.

In the combined use of these colored cyan couplers, the wavelength difference between the peaks of the two colored couplers is not less than about 10 nm, preferably not less than about 18 nm. These colored cyan couplers and the colorless cyan coupler are all incorporated in a red-sensitive layer and all react with an oxidation product of a p-phenylenediamine color developing agent to form a cyan dye image.

The colored cyan couplers of the present invention are illustrated below. Preferable examples of the colored cyan coupler having a main absorption in green region are illustrated by the couplers represented by the following general formula (I)



wherein R<sub>1</sub> represents an aryl group; R<sub>2</sub> represents an aryl group having at least one of an alkoxy carbonyl

group, an aryloxycarbonyl group, an alkylcarbonyl group or an arylcarbonyl group as a substituent; and preferable examples of the colored cyan coupler having a main absorption in the green region are illustrated by the couplers represented by the following general formula (II)



(II)

wherein  $R_3$  represents an alkyl group;  $R_4$  represents a monocyclic aryl group containing an aryloxycarbonyl group, an aryloxycarbonyl group, an alkylcarbonyl group or an arylcarbonyl group at the o-position with respect to the azo group.

In the above described general formula (I) and (II)  $R_1$  represents an aryl group (e.g., a phenyl group, a biphenyl group, a terphenyl group, a naphthyl group particularly an  $\alpha$ -naphthyl group, etc.) which can be unsubstituted or substituted with one or more of an alkyl group having 1 to 32 carbon atoms, a halogen atom, an alkoxy group having 1 to 32 carbon atoms, an acyloxy group, an aryloxycarbonyl group having 2 to 32 carbon atoms, an aryloxycarbonyl group, an acylamino group, an arylcarbonylamino group, a cycloalkylcarbonylamino group, an alkylamino group, an arylamino group, an N-alkylcarbamoyl group, an N-arylcarbamoyl group, an N-alkylureido group, an N-arylureido group, an alkylthio group, an arylthio group, an N-alkylsulfamoyl group, an N-arylsulfamoyl group, an alkylsulfonylamino group, an arylsulfonylamino group, a sulfo group, a carboxy group, a cycloalkylamino group, a cyclic amino group, an alkylcarbonyl group, an arylcarbonyl group, an alkylsulfonyl group, an arylsulfonyl group, a nitro group, a cyano group, a hydroxyl group, a mercapto group, a heterocyclic group, a sulfino group, a fluoroformyl group, a fluoro sulfonyl group, a perfluoroalkyl group, a perfluoroalkoxy group, a perfluoroacylaminogroup, a perfluoroalkylamino group, an N-perfluoroalkylcarbamoyl group, an N-perfluoroalkylureido group, a perfluoroalkylthio group, an N-perfluoroalkylsulfamoyl group, a perfluoroalkylsulfonyl group, or a perfluoroalkylsulfonyl group; and  $R_4$  represents a monocyclic aryl group (e.g., a phenyl group, a naphthyl group etc.) containing at least one of the same substituents at the o-position with respect to the azo group, as the substituents of  $R_2$ .

group, a naphthyoxy carbonyl group, etc.) in which the aryl group may be unsubstituted or substituted with one or more substituents as defined for  $R_1$ ; of an alkylcarbonyl group which may be unsubstituted or substituted with one or more substituents as defined for the aryloxycarbonyl group described above; and of an arylcarbonyl group which may be unsubstituted or substituted with one or more substituents as defined for the aryloxycarbonyl group described above;  $R_3$  represents an alkyl group having 1 to 32 carbon atoms which may be unsubstituted or substituted with one or more of an aryl group, an alkenyl group, an alkoxy group, an aryloxy group, an aryloxycarbonyl group, an aryloxycarbonyl group, an acylamino group, an arylcarbonylamino group, a cycloalkylcarbonylamino group, an alkylamino group, an arylamino group, an N-alkylcarbamoyl group, an N-arylcarbamoyl group, an N-alkylureido group, an N-arylureido group, an alkylthio group, an arylthio group, an N-alkylsulfamoyl group, an N-arylsulfamoyl group, an alkylsulfonylamino group, an arylsulfonylamino group, a sulfo group, a carboxy group, a cycloalkylamino group, a cyclic amino group, an alkylcarbonyl group, an arylcarbonyl group, an alkylsulfonyl group, an arylsulfonyl group, a nitro group, a cyano group, a hydroxyl group, a mercapto group, a heterocyclic group, a sulfino group, a fluoroformyl group, a fluoro sulfonyl group, a perfluoroalkyl group, a perfluoroalkoxy group, a perfluoroacylaminogroup, a perfluoroalkylamino group, an N-perfluoroalkylcarbamoyl group, an N-perfluoroalkylureido group, a perfluoroalkylthio group, an N-perfluoroalkylsulfamoyl group, a perfluoroalkylsulfonyl group, or a perfluoroalkylsulfonyl group; and  $R_4$  represents a monocyclic aryl group (e.g., a phenyl group, a naphthyl group etc.) containing at least one of the same substituents at the o-position with respect to the azo group, as the substituents of  $R_2$ .

Of the couplers represented by the above general formulae (I) and (II), examples of colored cyan couplers which are particularly preferred for the objects of the present invention are illustrated below.

A. Colored cyan couplers as described in U.S. Pat. 3,481,741, i.e., the compounds represented by the following general formula (III) which are particularly preferred as couplers of the above general formula (II) for the objects of the present invention



(III)

wherein  $R_5$  represents a branched alkyl group having 6 to 22 carbon atoms; and  $R_6$  represents a lower alkyl group having 1 to 6 carbon atoms.

Of these colored cyan couplers, particularly useful coupler compounds are shown below.



-continued



B. Colored cyan couplers as described in U.S. Pat. No. 3,459,552, i.e., the compounds represented by the following general formula (IV) which are particularly preferred as couplers of the general formula (I) for the objects of the present invention



45 wherein  $R_7$  represents a monocyclic aryl group having at least one alkoxy carbonyl group having 9 to 22 carbon atoms; and  $R_8$  represents a lower alkyl group having 1 to 6 carbon atoms.

Of these colored cyan couplers, particularly useful coupler compounds are shown below.



**-continued**



-continued

(14)



(15)



(16)



(17)



(18)



C. Colored cyan couplers described in U.S. Pat. No. 3,583,971, i.e., the compounds represented by the following general formula (V) which are particularly preferred as couplers of the above general formula (I) for the objects of the present invention



wherein R<sub>9</sub> represents a substituted or unsubstituted naphthalene ring residue connected to the amido group at the  $\alpha$ -position thereof; and X represents an aryl group having at least one alkoxy carbonyl group containing 2 to 22 carbon atoms.

Of these colored cyan couplers, particularly useful coupler compounds are shown below.



-continued

(23)



(24)



(25)



D. Colored cyan couplers as described in U.S. Pat. No. 3,034,892 and represented by the following general formula (VI) which are particularly preferred couplers of the above general formula (I) and (II) for the objects of the present invention

50

(VI)



wherein  $x$  represents an integer of 0 to 4;  $y$  represents 0 or 1;  $R_{10}$  represents an aryl group or an alkyl group having 6 to 22 carbon atoms (with the term aryl group including a phenyl group, an alkyl-substituted phenyl group), and  $R_{11}$  represents a straight-chain or branched-chain alkyl group having 1 to 4 carbon atoms.

60 65 Of these colored cyan couplers, particularly useful coupler compounds are shown below.



Preferred examples of colored cyan couplers having a main absorption in the blue region are illustrated by the couplers represented by the following general formulae (VII) and (VIII)



(VII)

5

10

20

25

35

40

45

50

55

60

65

15

wherein  $R_{12}$  represents an alkyl group; and  $R_{13}$  represents a monocyclic aryl group having an alkoxy carbonyl group or an aryloxycarbonyl group at the m- or p-position with respect to the azo group;



(VIII)

wherein  $R_{14}$  represents an alkyl group;  $R_{15}$  represents an alkyl group or an aryl group; and  $R_{16}$  represents a monocyclic aryl group having at least one of an alkoxy carbonyl group or an aryloxycarbonyl group as a substituent.

In the above general formula (VII) and (VIII)  $R_{12}$  represents an alkyl group (i.e., a straight chain or branched chain alkyl group having 1 to 32, conveniently 8 to 16 carbon atoms, which can be unsubstituted or substituted with; e.g., n-dodecyl, 2-methylpentyl, 1,3-dimethylbutyl, 2-ethylhexyl, 3-(n-dodecyloxy)propyl, 4-(3-pentadecylphenoxy)butyl, 2(2,4-di-t-pentylphenoxy)butyl, 3-(2-ethylhexyloxy)propyl, 2-2-[2-(2,4-di-t-pentylphenoxy)butyramido]phenyl ethyl, etc.;  $R_{13}$  represents a monocyclic aryl group containing the same substituents at the m- or p-position with respect to the azo group as the substituents as defined for  $R_4$ ;  $R_{14}$  represents an alkyl group (the same as defined for  $R_{12}$ ; e.g., preferably 2-ethylhexyl, n-octadecyl, methyl etc.);  $R_{15}$  represents an alkyl group (i.e., a straight chain or branched chain alkyl group having 1 to 32 carbon atoms) or an aryl group (i.e., a monocyclic aryl group, e.g., a phenyl group, a naphthyl group, etc.) which can be unsubstituted or substituted with; e.g., preferably methyl, n-octadecyl, 2-ethylhexyl, phenyl, 4-(4-t-butylphenoxy)phenyl, 4-[1-(2,4-di-t-pentylphenoxy)butyramido]phenyl,  $\alpha$ -phenethyl, 4-(2,4-di-t-pentylphenoxyacetamido)phenethyl, etc.; and  $R_{16}$  represents a monocyclic aryl group containing the same substituents as in  $R_4$  and  $R_{13}$ .

Preferred examples of colored cyan couplers having a main absorption in the blue region are illustrated by the compounds represented by the following general formulae (IX) to (XIII) which are particularly preferred as couplers of the above general formulae (VII) and (VIII) for the objects of the present invention



wherein  $R_{17}$  represents an alkyl group having 6 to 32 carbon atoms which can be further substituted with another substituent (a typical example including an n-hexyl group, an n-octyl group, a 2-ethylhexyl group, an n-dodecyl group, an n-octadecyl group, a  $\gamma$ -(n-dodecyloxy)-n-propyl group and a  $\gamma$ -(2,4-di-t-amylphenoxy)butyl group, etc.); and  $R_{18}$  represents an alkyl group having 1 to 20 carbon atoms;



wherein  $R_{17}$  and  $R_{18}$  are the same as defined above;



wherein  $R_{17}$  and  $R_{18}$  are the same as defined above;





(XIII)

tuted with other substituents).

Of the colored cyan couplers represented by the general formula (IX), particularly useful coupler compounds are shown below.

(31)



(32)



Of the colored cyan couplers represented by the following general formula (X), a particularly useful coupler compound is shown below.

35

40



45

Of the colored cyan couplers represented by the following general formula (XI), particularly useful coupler compounds are illustrated below.

(34)



(35)



-continued

(36)



(37)



(38)



(39)



(40)



Of the colored cyan couplers represented by the general formula (XII), particularly useful coupler compounds are:

(41)



(42)



60

65

Of the colored cyan couplers represented by the general formula (XIII), a particularly useful coupler compound is



As the colorless cyan couplers of the present invention, a wide variety of couplers can be used. For example, coupler compounds having 15 to 44 carbon atoms and having substantially no absorption in the visible light range can be selected from conventionally known cyan couplers (for example, as described in W. Pelz, *Mitteilungen aus den Forschungs-Laboratorien der Agfa Leverkusen Munchen III*, pp. 156-174 (1961)). In particular, coupler compounds represented by the following general formula (XIV) or (XV) provide good results,



wherein R<sub>23</sub> and R<sub>24</sub> each represents a hydrogen atom, an alkyl group (preferably a straight or branched chain alkyl group having 1 to 30 carbon atoms), a cyclic alkyl group (e.g., a cyclohexyl group, a norbornyl group, etc.), an aryl group (e.g., a phenyl group, a terphenyl group, a naphthyl group, etc.), a heterocyclic group (e.g., a benzimidazolyl group, a benzothiazolyl group, etc.), or in combination the non-metallic atoms necessary for forming a heterocyclic ring such as morpholine or piperidine, the alkyl group, aryl group, heterocyclic group or the like may be substituted with a halogen atom, a nitro group, a hydroxy group, a carbonyl group, an amino group (e.g., an amino group, an alkylamino group, a dialkylamino group, an anilino group, an N-alkylanilino group, etc.), an aryl group, an alkoxy carbonyl group, an aryloxycarbonyl group, an amido group (e.g., an acetamido group, a butyramido group, an ethylsulfonamido group, an N-methyl-benzamido group, an N-propylbenzamido group, a 4-t-butylbenzamido group, etc.), a carbamyl group (e.g., a carbamyl group, an N-octadecylcarbamyl group, an N,N-dihexylcarbamyl group, an N-methyl-N-phenylcarbamyl group, a 3-pentadecylphenylcarbamyl group, etc.), a sulfamyl group (e.g., an N-propylsulfamyl group, an N-tolylsulfamyl group, etc.), an alkoxy group (e.g., an ethoxy group, an octadecoxy group, etc.), an aryloxy

- 15 group (e.g., a phenoxy group, a tolyloxy group, a naphthoxy group, etc.), a sulfo group, a sulfonyl group (e.g., a methylsulfonyl group, an octadecylsulfonyl ethoxysulfonyl group, a decoxysulfonyl group, a phenylsulfonyl group, a tolylsulfonyl group, a phenoxy sulfonyl group, etc.), or the like; R<sub>27</sub> represents a hydrogen atom, a halogen atom (e.g., a chlorine atom, a bromine atom, etc.) an alkyl group (e.g., having 1 to 20 carbon atoms such as a methyl group, a dodecyl group, etc.), an aryl group, a heterocyclic group, an amino group (e.g., an amino group, an alkylamino group, an arylamino group, etc.), a carbonamido group (e.g., an alkylcarbonamido group, an arylcarbonamido group, a heterocyclic carbonamido group, etc.), a sulfonamido group (e.g., an alkylsulfonamido group, an arylsulfonamido group, a heterocyclic sulfonamido group, etc.), a sulfamyl group (e.g., an alkylsulfamyl group, an arylsulfamyl group, a heterocyclic sulfamyl group, etc.), a carbamyl group (e.g., an alkylcarbamyl group, an arylcarbamyl group, a heterocyclic carbamyl group, etc.), an ureido group (e.g., an N-alkylureido group, an N-arylureido group, etc.), where the alkyl group, aryl group or heterocyclic group can contain the substituents described above with respect to R<sub>23</sub> and R<sub>24</sub>, R<sub>25</sub>, R<sub>26</sub>, R<sub>28</sub>, R<sub>29</sub> and R<sub>30</sub> each represents the groups as described with respect to R<sub>27</sub>, and further represents a halogen atom (e.g., a chlorine atom, a bromine atom, etc.) or an alkoxy group (e.g., a methoxy group, a dodecyloxy group, etc.), X and Y each represents a hydrogen atom, a group capable of being eliminated upon coupling (e.g., a halogen atom, a thiocyanato group, an alkoxy group, an aryloxy group, etc.), or X may be a cyclic imido group (e.g., a maleimido group, a succimido group, a 1,2-dicarboxyimide group, a phthalimido group, etc.) or a residue capable of releasing a restrainer upon development (e.g., an arylmonothio group, a heterocyclic thio group, a 2-benzotriazole group, a 2-benzodiazole group, and arylsulfinyl group, etc.).
- 55 More specifically, those colorless cyan couplers as described in U.S. Pat. Nos. 2,369,929, 3,591,383, 3,458,315, 2,474,293, 2,908,573, 3,419,390, 3,476,563, 3,253,924, 2,434,272, 3,516,831, 3,311,476, 2,698,974, 3,227,554, 3,701,783, 60 3,617,291, 3,622,328, 2,908,573, Japanese Pat. Publication Nos. 5547/64, 6993/70, 12988/63, 18145/63, 28836/70, 19032/71, Japanese Pat. Application Nos. 35379/73, 69383/73, West German Pat. OLS Nos. 2,216,578, 2,163,811, etc. are preferred as colorless cyan couplers.
- 65 Further, specific compounds particularly preferred as the colorless cyan couplers are illustrated by the following.

(44)



(45)



(46)



(47)



(48)



(49)



(50)



(51)



(52)

-continued



(53)



(54)



(55)



(56)



(57)



(58)



-continued

(59)



(60).



(61)



(62)



(63)



(64)



-continued

Three couplers of the present invention, i.e., a colored cyan coupler having a main absorption in the blue region, a colored cyan coupler having a main absorption in the green region and a colorless cyan coupler, as described before are incorporated in a red-sensitive layer and are desirably incorporated in the same red-sensitive layer of the color photographic light-sensitive material. However, it is possible to incorporate two of them in the same red-sensitive layer and the third in a different red-sensitive layer. Also, it is possible to incorporate the couplers independently in three different red-sensitive layers.

On the other hand, the following configurations are suitable for the light-sensitive material of the present invention. That is, in a color photographic light-sensitive material having a stratum structure comprising a red-sensitive layer, a green-sensitive layer and a blue-sensitive layer, the red-sensitive layer is constituted as described in detail before, the green-sensitive layer can contain a colorless magenta coupler, a colored magenta coupler, a DIR magenta coupler and a non-coloring DIR compound as described in U.S. Pat. Nos. 3,379,529, 3,639,417, 3,297,445, 3,632,345, and the blue-sensitive layer can contain a colorless yellow coupler, a DIR yellow coupler and the above described non-coloring DIR compound.

With respect to the use of DIR couplers and/or DIR compounds in the red-sensitive layer, the green-sensitive layer and the blue-sensitive layer of the color light-sensitive material of the present invention, the processes described in U.S. Pat. No. 3,703,375, Japanese Patent Publication Nos. 28836/70, 19034/71, Japanese Pat. Application Nos. 50051/73, 68892/73, West German Pat. OLS Nos. 2,060,196, 2,322,165, etc. can be utilized. Also, with respect to the structure of auxiliary layers upon use of DIR couplers and/or DIR compounds, the processes described in U.S. Pat. 3,737,317, Japanese Pat. Application Nos. 73445/73, 103542/73 and 113633/73 are preferably used.

The amount of each of the colored cyan coupler having a peak in the blue light absorption region and of the colored cyan coupler having a peak in the green light absorption region in general, can range from about 0.02 to about 2 mols per 1 mol of the colorless cyan coupler. Preferably, the amounts range from 0.05 to 1.5 mols per mol of the colorless cyan coupler. A suitable molar ratio of silver to the colorless cyan coupler and the two types of colored cyan couplers is about 4:1 to 100:1, preferably 4:1 to 50:1.

When the molar proportion of the colored cyan coupler having an absorption peak in the blue light region

to the colored cyan coupler having an absorption peak in the green light region is within the range of about 10:1 to 1:10, the effect of the present invention can be observed. However, in order to enhance the effect of the present invention to the fullest, a preferred molar ratio ranges from 2:1 to 1:2.

Useful magenta couplers which can be used in the present invention are those magenta couplers described in U.S. Pat. Nos. 3,253,924, 3,516,831, Japanese Pat. Laid-Open No. 5482/72, U.S. Pat. Nos. 2,600,788, 3,558,319, 2,439,098, Japanese Pat. Application No. 21454/73, British Pat. No. 1,293,640, U.S. Pat. 3,468,666, 3,419,391, Japanese Pat. Application No. 56050/73, U.S. Pat. Nos. 3,311,476, 3,061,432, Japanese Pat. Publication No. 2016/69, Japanese Pat. Application No. 33238/73, U.S. Pat. Nos. 3,148,062, 2,908,573, Japanese Pat. Application Nos. 35379/73, 69383/73, Japanese Pat. Publication No. 19032/71, German Pat. OLS No. 2,216,578, U.S. Pat. Nos. 3,227,554, 3,701,783, 3,617,291, etc. and, even more useful colored magenta couplers are those magenta couplers described in U.S. Pat. Nos. 2,434,272, 3,703,375, Japanese Pat. Publication No. 2016/69, U.S. Pat. No. 3,476,564, Japanese Pat. Application No. 45971/73, U.S. Pat. No. 3,476,560, etc. Illustrative examples of particularly useful colored magenta couplers are 1-(2,4,6-tri-chlorophenyl)-3-[3-(2,4-di-tert-amylphenoxyacetamido)benzamido]-4-(4-methoxyphenylazo)-2-pyrazolin-1-(2,4,6-trichlorophenyl)-3-3-[ $\alpha$ -(2,4-di-tert-amylphenoxy)-butyramido]benzamido-4-(4-methoxyphenylazo)-2-pyrazolin-5-one, 1-(2,4,6-trichlorophenyl)-3-(2-chloro-5-tetradecanoylamidoanilino)-4-(4-hydroxy-3-methylphenylazo)-2-pyrazolin-5-one.

Yellow couplers which can be in the present invention are described in U.S. Pat. No. 3,253,924, Japanese Pat. Publication No. 18735/64, U.S. Pat. Nos. 2,728,658, 3,265,506, 3,369,895, 3,582,322, 3,725,072, West German Pat. OLS Nos. 1,956,281, 2,162,899, U.S. Pat. Nos. 3,408,194, 3,447,928, 3,415,652, West German Pat. OLS No. 2,213,461, Japanese Pat. Laid-Open No. 3039/73, British Pat. No. 1,204,680, U.S. Pat. Nos. 2,908,573, 3,510,306, 3,658,544, 3,730,722, Japanese Pat. Application Nos. 35379/73, 69383/73, West German Pat. OLS No. 2,216,578, U.S. Pat. Nos. 3,148,062, 3,227,554, 3,701,783, etc.

The couplers used in the present invention can be dissolved in an oily solvent such as tricresylphosphate and dispersed and emulsified in a hydrophilic colloid aqueous solution, such as a gelatin aqueous solution, in

the presence of a suitable surface active agent. In this case, the couplers are desirably emulsified together with a colorless cyan coupler. However, it is also possible to separately emulsify them and then mix the individual coupler dispersions. Suitable processes for dispersion and emulsification are given in the foregoing patents.

The photographic light-sensitive material of the present invention desirably contains, as a red-sensitive layer, a silver halide emulsion layer containing a colored cyan coupler-containing emulsion. However, the present invention is not limited only to this embodiment.

A silver halide emulsion is usually prepared by mixing a solution of a water-soluble silver salt (e.g., silver nitrate, etc.) with a solution of a water-soluble halide (e.g., potassium bromide, etc.) in the presence of a water-soluble high polymer such as gelatin. Silver bromoiodide, silver chlorobromoiodide, silver bromide, etc. are usually used as the silver halide. The weight ratio of silver to the hydrophilic colloid generally ranges from about 1:10 to 5:1, preferably 1:5 to 3:1 in the emulsion to be used in the present invention. These silver halide grains can be prepared using known conventional processes. For example they can be prepared by the so-called single- or twin-jet process, controlled twin jet process, or the like. The mean grain size of the silver halide preferably ranges from 0.1  $\mu$  to 2.0  $\mu$ . These photographic emulsions are also described in C. E. K. Mees & T. H. James; *The Theory of Photographic Process*, Macmillan Co., New York (1966), P. Grafkides; *Chimie Photographique*, Paul Montel, Paris (1957), or similar references, and can be prepared using various processes commonly known, such as an ammonia process, a neutral process, an acidic process, etc.

After the formation of the silver halide grains, the system is washed with water to remove water-soluble salts (for example, potassium nitrate when silver bromide is formed from silver nitrate and potassium bromide) from the system. Then, heat treatment is effected in the presence of a chemical sensitizer such as sodium thiosulfate, N,N,N'-trimethylthiourea, a thiocyanate complex salt or thiosulfate complex salt of monovalent gold, stannous chloride, hexamethylenetetramine, etc. to increase the sensitivity without coarsening the grains. General processes for chemical sensitization and chemical sensitizers which can be used are described in the above-described references and in U.S. Pat. Nos. 1,574,944, 2,278,947, 2,399,083, 2,410,689, 2,448,060, 2,487,850, 2,518,698, 2,521,925, 2,521,926, 2,491,973, 2,540,806, 2,566,245, 2,566,263, 2,419,975, 3,189,458, 3,297,446, and 3,501,313.

Illustrative hydrophilic colloids which can be used as a binder for the silver halide are, e.g., gelatin, colloidal albumin, casein, cellulose derivatives (e.g., carboxymethyl cellulose, hydroxyethyl cellulose, etc.), saccharide derivatives (e.g., agaragar, sodium alginate, starch derivatives, etc.) synthetic hydrophilic colloids (e.g., polyvinyl alcohol, poly-N-vinyl pyrrolidone, acrylic acid copolymers, polyacrylamide, the derivatives or partially hydrolyzed products thereof, etc.). If desired, a compatible mixture of two or more of these binders can be used. Of these, the most generally used binder is gelatin. Gelatin can be replaced, partly or completely, by a synthetic high molecular substance, by a so-called gelatin derivative (prepared by processing and modify-

ing gelatin with a compound having a group capable of reacting with the functional groups contained in the gelatin molecule (i.e., amino groups, imino groups, hydroxy groups or carboxy groups)), or by a graft polymer prepared by grafting a molecular chain of another high molecular substance onto gelatin.

The above-described red-sensitive photographic emulsions are provided with a red sensitivity by adding panchromatically sensitizing dyes as described in U.S. Pat. Nos. 3,511,664, 3,522,052, 3,527,641, 3,615,613, 3,615,632, 3,615,641, 3,617,293, 3,617,295, 3,635,721, 3,694,217, 3,743,510, etc. A green sensitivity can be provided to the green-sensitive layers by employing green sensitizing dyes as described in U.S. Pat. Nos. 2,688,545, 2,912,329, 3,397,060, 3,615,635, 3,628,964, 3,793,020, 3,656,959, 3,769,301, 3,814,609, West German Pat. OLS No. 2,121,780, Japanese Pat. Publication Nos. 4936/68, 14030/69, etc., and a blue sensitivity can be provided to the blue-sensitive layers by employing blue sensitizing dyes as described in U.S. Pat. Nos. 2,493,748, 2,519,001, 2,977,229, 3,480,434, 3,672,897, 3,703,377, etc.

To the above-described photographic emulsion can be added various compounds in order to prevent a reduction in sensitivity and formation of fog during production, during storage or during processing of the light-sensitive material. An extremely large number of such compounds is well known in the art, such as heterocyclic compounds including 4-hydroxy-6-methyl-1,3,3a,7-tetraazaindene, 3-methylbenzothiazole and 1-phenyl-5-mercaptopurine, mercury-containing compounds, mercapto compounds, metal salt compounds, and the like.

Examples of suitable compounds are described in C. E. K. Mees & T. H. James; *The Theory of the Photographic Process*, 3rd. Ed. p. 344-6 Macmillan, New York (1966), and the original literature references cited therein and are also described in U.S. Pat. Nos. 1,758,576, 2,110,178, 2,131,038, 2,173,628, 2,697,040, 2,304,962, 2,324,123, 2,394,198, 2,444,605-8, 2,566,245, 2,694,716, 2,697,099, 2,708,162, 2,728,663-5, 2,476,536, 2,824,001, 2,843,491, 2,886,437, 3,052,544, 3,137,577, 3,220,839, 3,226,231, 3,236,652, 3,251,691, 3,252,799, 3,287,135, 3,326,681, 3,420,668, and 3,622,339, and British Pat. Nos. 893,428, 403,789, 1,173,609, and 1,200,188.

Surface active agents alone or in combination can be added to the above-described photographic emulsion. They are used as a coating aid but, in some cases, they are used for the improvement of sensitization and photographic properties, antistatic purposes and the prevention of adhesion.

These surface active agents can be classified into natural surface active agents such as saponin; nonionic surface active agents such as alkylene oxide compounds, glycerin compounds, glycidol compounds, etc.; cationic surface active agents such as higher alkyl amines, quaternary ammonium salts, heterocyclic compounds (e.g., pyridine, etc.), phosphonium compounds, sulfonium compounds, etc.; anionic surface active agents having an acidic group such as a carboxylic acid group, a sulfonic acid group, a phosphoric acid group, a sulfuric ester group, a phosphoric acid ester group, etc.; and amphoteric surface active agents such as aminoacids, aminosulfonic acids, aminoalcohol sulfuric or phosphoric esters, etc.

Examples of suitable surface active compounds are described in, e.g., U.S. Pat. Nos. 2,271,623, 2,240,472, 2,288,226, 2,739,891, 3,068,101, 3,158,484, 3,201,253, 3,210,191, 3,294,540, 3,415,649, 3,441,413, 3,442,654, 3,475,174, 3,545,974, West German Patent OLS No. 1,942,665, British Pat. Nos. 1,077,317, 1,198,450, etc. and in, e.g., Ryohei Oda; *Synthesis and Application of Surface Active Agents*, Maki Shoten, (1964), A.W. Schwartz et al; *Surface Active Agents* Interscience Publication Inc., (1958), J. P. Sisley and P. J. Wood; *Encyclopedia of Surface Active Agents*, vol. 2, Chemical Publishing Co., (1964), and the like.

In order to increase the strength of coated layers a hardener can be incorporated in the above-described photographic emulsion. Illustrative examples of hardeners are, for example, ketone compounds (e.g., diacetyl, cyclopentanedione, etc.), compounds having a reactive halogen (e.g., bis(2-chloroethylurea), 2-hydroxy-4,6-dichloro-1,3,5-triazine, the compounds described in U.S. Pat. Nos. 3,288,775, 2,732,303, British Pat. Nos. 974,723, 1,167,207, etc.), compounds having a reactive olefin such as divinylsulfone, 5-acetyl-1,3-diacryloylhexahydro-1,3,5-triazine, those compounds described in U.S. Pat. Nos. 3,635,718, 25 3,232,763, British Pat. Nos. 994,896, etc.; isocyanates as described in U.S. Patents 3,103,437; aziridine compounds as described in U.S. Pat. Nos. 3,017,280, 2,983,611, etc.; acid derivatives as described in U.S. Pat. Nos. 2,725,294, 2,725,295, etc.; carbodiimide compounds as described in U.S. Pat. No. 3,100,704, etc.; epoxy compounds as described in U.S. Pat. No. 3,091,537, etc.; isoxazole compounds as described in U.S. Pat. Nos. 3,321,313 and 3,543,292; halocarboxy-aldehydes such as mucochloric acid, etc.; dioxane derivatives such as dihydroxydioxane, dichlorodioxane, etc.; and inorganic hardening agents such as chromium alum, zirconium sulfate, etc. Also, precursors of the above-described compounds such as the alkali metal bisulfite-aldehyde adducts, hydantoin methylol compounds, primary aliphatic nitroalcohols, etc. can be used in place of the above-described compounds.

The photographic emulsion layer used in the present invention can contain a light absorbent and a filtering dye as described in U.S. Pat. No. 3,547,640, etc. If 45 desired, the dye may be mordanted.

This photographic emulsion can be coated on a support conventionally employed for photographic light-sensitive materials, such as a cellulose nitrate film, a cellulose acetate film, a cellulose acetate butyrate film, a cellulose acetate propionate film, a polystyrene film, a polyethylene terephthalate film, a polycarbonate film, etc. These supports can be transparent and also colored by the addition of a dye or a pigment. Also, those supports having a colored subbing layer coated thereon can be used as a support. A suitable coating amount of the silver halide emulsion ranges from about 10 to 150 mg of silver per 100 cm<sup>2</sup> of the support.

This photographic emulsion can be coated using a variety of coating methods including a dip-coating method, an air knife-coating method, a curtain-coating method and an extrusion coating method using a hopper as described in U.S. Pat. No. 2,681,294. If desired, two or more layers can be coated at the same time according to the method described in U.S. Pat. Nos. 2,761,791, 3,508,947, 2,941,898, 3,526,528, etc.

The color photographic light-sensitive material of the present invention is completed by coating, in sequence,

a green-sensitive emulsion layer, a yellow filter layer and a blue-sensitive emulsion layer on the aforesaid red-sensitive emulsion layer coated on the support. The coating sequence of each emulsion layer can be altered. The color photographic material of the present invention can further contain usual light-insensitive layers (e.g., a protective layer, a filter layer, an interlayer, an anti-halation layer, a subbing layer, a backing layer, etc.).

10 The color photographic light-sensitive material of this invention can be exposed for about 10<sup>-4</sup> to 10 seconds using sunlight, a tungsten lamp or a flash lamp. Ordinary color photographic processings can be applied to the color photographic light-sensitive material of the present invention. The photographic processings can be effected at a temperature of from about 20°C or lower to about 60°C or higher.

15 Suitable color developers are an alkaline aqueous solution having a pH of not less than about 8, preferably 9 to 13 and containing an aromatic primary amine developing agent. Typical examples of aromatic primary amine developing agents are p-phenylenediamine derivatives and the inorganic acid salts thereof such as N,N-diethyl-p-phenylenediamine, 2-amino-5-diethylaminotoluene, 2-amino-5-(N-ethyl-N-laurylaminol)toluene, 4-[N-ethyl-N-(β-hydroxyethyl)amino]aniline, 3-methyl-4-amino-N-ethyl-N-(β-hydroxyethyl)aniline, etc.; 4-amino-3-methyl-N-ethyl-N-(β-methanesulfoamidoethyl)aniline sesquisulfate monohydrate as described in U.S. Pat. No. 2,193,015; N-(2-amino-5-diethylaminophenylethyl)methanesulfonamide sulfate as described in U.S. Pat. No. 2,592,364; N,N-dimethyl-p-phenylenediamine hydrochloride; 3-methyl-4-amino-N-ethyl-N-methoxyethylaniline as described in Japanese Pat. Laid-Open No. 64933/73; and the like.

20 These color developing agents are described in detail in, e.g., L.F.A. Mason; *Photographic Processing Chemistry*, pp. 226-229 Focal Press, London, (1966).

25 Also, these color developing agents can be used in combination with 3-pyrazolidones.

30 After development, the silver images are converted to silver halide by bleaching and then the bleached silver dissolved away by fixing. Bleaching and fixing can be effected sequentially or at the same time using a bleach-fixing bath.

35 In the bleaching solution are incorporated various oxidizing agents. Typical examples of oxidizing agents are ferricyanides (e.g., a potassium salt, a sodium salt, an ammonium salt, etc.), water-soluble quinones (e.g., quinone, sulfophenylquinone, chloroquinone, methoxyquinone, 2,5-dimethoxyquinone, methylquinone, etc.), dichromates, nitrosophenol, water-soluble copper (II) salts (cupric chloride, cupric nitrate, copper (II) sulfate, etc.), simple water-soluble cobalt (III) (e.g., cobalt (III) chloride, ammonium cobalt (III) nitrate, etc.), a complex salt between a multivalent cation such as iron (III), cobalt (III), copper (II), etc. and an organic acid (e.g., a metal complex salt of ethylenediaminetetraacetic acid, nitrilotriacetic acid, iminodiacetic acid, N-hydroxyethylmethylenediaminetriacetic acid or a like aminopolycarboxylic acid, malonic acid, tartaric acid, malic acid, diglycolic acid or dithioglycolic acid; 2,6-dipicolinic acid-copper complex salt; etc.), peracids (e.g., an alkylperacid, a persulfate, permanganate, hydrogen peroxide, etc.), hypochlorite, chlorine, bromine, and the like.

These various bleaching agents are described in Japanese Pat. Publication Nos. 14035/70, 13944/66, 11068/66, U.S. Pat. Nos. 2,507,183, 2,529,981, 2,625,477, 2,748,000, 2,810,648, 2,705,201, British Pat. Nos. 982,984, 1,014,396, 1,032,024, 777,635, 717,139, 1,111,313, etc.

The fixing solution contains a suitable silver halide solvent such as a water-soluble thiosulfate (e.g., a potassium salt, a sodium salt, an ammonium salt, etc.), a water-soluble thiocyanate (e.g., sodium salt, potassium salt, ammonium salt, etc.), a water-soluble sulfur-containing diol fixing agent (e.g., 3-thia-1,5-pentanediol, 3,6-dithia-1,8-octanediol, 3,6,9-trithia-1,1,1-undecanediol, etc.), a water-soluble sulfur-containing organic dibasic acid (e.g., ethylenebisthioglycolic acid, thioglycolic acid, etc.) or the alkali metal salt of such a dibasic acid.

Ordinary additives for each processing solution can be incorporated in the color developer, the bleaching solution and the fixing solution.

The processing steps can include, in addition to the above-described three basic steps of developing, bleaching and fixing, other steps (for example, a stopping bath, a hardening bath, a stabilizing attained washing, etc.), if desired.

According to the present invention, a color print with good color reproduction can be obtained. That is, suitable color correction of a cyan dye in a color negative image can be obtained through sufficient masking and, as a result, color stain-free color prints having distinct red and yellow images can be obtained. As a result, colored cyan couplers can be selected from a wide range of compounds taking into consideration only the difference in the absorption peaks. Therefore, the present invention is advantageous in designing a color photographic emulsion.

The present invention is illustrated in greater detail by reference to the following examples. Unless otherwise indicated, all parts, percents, ratios and the like are by weight.

#### EXAMPLE 1

To 1,000 g of a high speed negative silver bromoiodide emulsion containing 6.5 g of silver bromoiodide (containing 6.0 mol% of silver iodide) and 10 g of gelatin were added, in sequence, 200 cc of a 0.03% methanol solution of the following optical sensitizer, 20 cc of a 1% aqueous solution of 5-methyl-7-hydroxy-1,3,4-triazaindolizine, 450 g of the following Emulsion (1) containing a colorless cyan coupler (Compound 44) and, as a gelatin hardener, 50 cc of a 2% aqueous solution of 2-hydroxy-4,6-dichloro-s-triazine sodium salt, to prepare a red-sensitive emulsion.



#### EMULSION (1)

A mixture comprising 110 cc of ethyl acetate, 80 g of Compound 44 (colorless cyan coupler), 5 g of sodium p-dodecylbenzene sulfonate and 65 cc of tricresylphosphate was melted at 60°C and added to 1,000 cc of a 10% aqueous solution of gelatin previously maintained at 60°C, followed by stirring for 20 minutes using a

mixer for emulsification. Thus, Emulsion (1) was prepared.

The red-sensitive color emulsion obtained above was coated on a cellulose triacetate support having a subbing layer thereon, at a coverage of 20 mg/100 cm<sup>2</sup> of silver to prepare Color Photographic Film (A).

Film (A) was exposed to red light through a conventional gray wedge and subjected to the following color development processing.

10 The density of the developed film was measured through a red, green or blue filter to obtain the characteristic curves shown in FIG. 2.

From FIG. 2, it can be seen that, when only the colorless cyan coupler is used, a cyan dye having side-absorptions in the blue and green regions is formed.

| Development Processing Steps | Temperature | Time    |
|------------------------------|-------------|---------|
| Color Development            | 24°C        | 12 min. |
| Stopping Solution Bath       | "           | 4       |
| Hardening Bath               | "           | 4       |
| 20 Washing                   | "           | 4       |
| Bleaching Bath               | "           | 6       |
| Washing                      | "           | 4       |
| Fixing Bath                  | "           | 8       |
| Washing                      | "           | 8       |
| Drying                       | "           |         |

25 The processing solutions used had the following formulations.

|                                                                |         |  |
|----------------------------------------------------------------|---------|--|
| Color Developer Solution                                       |         |  |
| Benzyl Alcohol                                                 | 5 ml    |  |
| Sodium Hydroxide                                               | 0.5 g   |  |
| 30 Diethylene Glycol                                           | 3 ml    |  |
| Sodium Hexametaphosphate                                       | 2 g     |  |
| Sodium Sulfite                                                 | 2 g     |  |
| Potassium Bromide                                              | 2 g     |  |
| 4-Amino-3-methyl-N-ethyl-N-(β-hydroxyethyl)aniline Monosulfate | 5 g     |  |
| 35 Metaboric Acid                                              | 0.5 g   |  |
| Sodium Metaborate (tetrahydrate)                               | 77 g    |  |
| Water to make                                                  | 1 liter |  |

#### Stopping Bath

|                     |         |  |
|---------------------|---------|--|
| 40 Sodium Acetate   | 30 g    |  |
| Glacial Acetic Acid | 8 ml    |  |
| Water to make       | 1 liter |  |

#### Hardening Solution

|                          |         |  |
|--------------------------|---------|--|
| Sodium Hexametaphosphate | 1 g     |  |
| Borax (pentahydrate)     | 20 g    |  |
| Formalin (37%)           | 10 ml   |  |
| Water to make            | 1 liter |  |

#### Bleaching Solution

|                        |      |  |
|------------------------|------|--|
| Potassium Ferrocyanide | 8 g  |  |
| Potassium Ferricyanide | 30 g |  |
| Potassium Bromide      | 20 g |  |
| Borax (pentahydrate)   | 15 g |  |
| Boric Acid             | 5 g  |  |

#### Disodium Ethylenediaminetetraacetate

|               |         |  |
|---------------|---------|--|
| 65 Dihydrate  | 1 g     |  |
| Water to make | 1 liter |  |

#### Fixing Solution

|                          |     |  |
|--------------------------|-----|--|
| Sodium Hexametaphosphate | 1 g |  |
| Sodium Sulfite           | 5 g |  |

|                    |         |
|--------------------|---------|
| Sodium Thiosulfate | 150 g   |
| Acetic Acid        | 8 ml    |
| Water to make      | 1 liter |

Next, Emulsion (2) was prepared in the same manner as Emulsion (1) except for using 65 g of Compound (44) and 15 g of Compound (21), as a colored cyan coupler of the invention having an absorption in a long wavelength region represented by the general formula (V), in combination in place of Compound (44). The spectral absorption spectrum of Compound (21) is shown in FIG. 1.

A photographic emulsion was prepared in the same manner as described above except for using Emulsion (2), and Color Photographic Film (B) was prepared therefrom. Film (B) was exposed, development-processed and subjected to densitometry in absolutely the same manner as described above, to obtain the characteristic curves as shown in FIG. 3.

From FIG. 3, it can be seen that, when a colored cyan coupler having an absorption in the long wavelength region is used in combination with a colorless cyan coupler, the masking effect on the side-absorption in the blue region of the dye formed is insufficient although the masking effect on the side-absorption in the green region is sufficient.

Next, Emulsion (3) was prepared in the same manner as Emulsion (1) except for using 80 g of Compound (35) as a colored cyan coupler of the present invention having an absorption in a short wavelength region in place of Compound (44). The spectral absorption spectrum of Compound (35) is also shown in FIG. 1. A photographic emulsion was prepared in the same manner as described above except for using 70 g of Emulsion (3) and 380 g of Emulsion (1). Thus, Color Photographic Film (C) was obtained. Film (C) was exposed, development-processed and subjected to densitometry in absolutely the same manner as described above, to obtain the characteristic curves shown in FIG. 4.

From FIG. 4, it can be seen that, when a colored cyan coupler having an absorption in a short wavelength region is used in combination with a colorless cyan coupler, the masking effect on the side-absorption in the green region of the cyan dye formed is insufficient although the masking effect on the side-absorption in the blue region is sufficient.

Next, Emulsion (4) was prepared in the same manner as Emulsion (1) except for using 65 g of a Compound (44) as a colorless cyan coupler, 15 g of a Compound (21), as a colored cyan coupler having an absorption in a short wavelength region, and 11 g of Compound (35) as a colored cyan coupler having an absorption in a short wavelength region. A photographic emulsion was prepared in the same manner as described above except for using Emulsion (4), and Color Photographic Film (D) was obtained therefrom. Film (D) was exposed, development-processed and subjected to densitometry in absolutely the same manner as described above, to obtain the characteristic curves as shown in FIG. 5.

As is shown in FIG. 5, the side-absorptions of the formed cyan dye in the blue and green regions are sufficiently masked by using a colored cyan coupler having an absorption in a short wavelength region and a colored cyan coupler having an absorption in a long wavelength region, in combination.

#### EXAMPLE 2

Emulsion (5) was prepared in the same manner as Emulsion (1) except for replacing the cyan couplers by

12 g of a colored cyan coupler (Compound (41), 14 g of a colored cyan coupler (Compound (4)) and 65 g of a colorless cyan coupler (Compound (44)). As is shown in FIG. 1, the colored cyan coupler (Compound (41)) has a main absorption in the blue region, with an absorption peak at 485 m $\mu$ . On the other hand, colored cyan coupler (Compound (4)) has a main absorption in the green region, with the absorption peak at 503 m $\mu$ . The difference in the wavelength between both of the peaks is 18 m $\mu$ . A photographic emulsion was prepared in the same manner as described in Example 1 except for using Emulsion (5) to obtain Color Photographic Film (E). Further, Emulsion (6) was prepared in the same manner as Emulsion (5) except for completely replacing the colored cyan couplers by Compound (41). Separately, Emulsion (7) was obtained in the same manner as Emulsion (5) except for completely replacing the colored cyan couplers by Compound (4). Color Photographic Films (F) and (G) were obtained in the same manner using Emulsions (6) and (7), respectively.

Films (E), (F) and (G) were exposed, development-processed and subjected to densitometry in absolutely the same manner as in Example 1. As a result, the gammas of the cyan, magenta and yellow components of the image density appearing in characteristic curves were obtained.

| Film | Red-light Photometry Gamma (Cyan) | Green-light Photometry Gamma (Magenta) | Blue-light Photometry Gamma (Yellow) |
|------|-----------------------------------|----------------------------------------|--------------------------------------|
| E    | 1.05                              | 0.04                                   | 0.02                                 |
| F    | 1.00                              | 0.12                                   | 0.01                                 |
| G    | 1.08                              | 0.02                                   | 0.07                                 |

Gamma = slope of characteristic curve at a linear portion

The gamma of the cyan dye image of all of Films (E), (F) and (G) measured using red light photometry was almost 1. However, with Film F containing only two couplers, a colored cyan coupler (compound 41) having a main absorption in the blue region and a colorless cyan coupler (Compound (44)), the gamma of the magenta image in the green light region was as large as 0.12 showing that masking was insufficient, although the gamma of the yellow image in the blue region was 0.01 which was substantially zero showing that masking in this region was sufficient. On the other hand, with Film (G) containing only two couplers, a colored cyan coupler (Compound (4)) having a main absorption in the green region and a colorless cyan coupler (Compound (44)), the gamma of the yellow image in the blue region was as large as 0.07 showing that masking was insufficient, although the gamma of the magenta image in the green region was 0.02 which was nearly zero showing that masking at this region was sufficient.

With Film (E) containing three couplers, a colored cyan coupler (Compound (41)) having a main absorption in the blue region, a colored cyan coupler (Compound (4)) having a main absorption in the green region and a colorless cyan coupler (Compound (44)), the gamma value of the yellow image in the blue region and that of the magenta image in the green region were 0.02 and 0.04, respectively, which were both nearly zero showing that masking was sufficient in both regions.

That is, the above-described results show that unnecessary absorption components can be sufficiently masked as long as the difference in wavelength of the peaks of absorption of both of the colored couplers is

18 nm, as is shown by the peak difference between the Colored Cyan Coupler (41) having a main absorption in a blue region shorter than 490 nm and the Colored Cyan Coupler (Compound (4)) having a main absorption in the green region lying in a longer side.

While the invention has been described in detail and with reference to specific embodiments thereof, it will be apparent to one skilled in the art that various changes and modifications can be made therein without departing from the spirit and scope thereof.

What is claimed is:

1. A color photographic light-sensitive material comprising a support having thereon at least one silver halide emulsion and the light-sensitive material containing a colored cyan coupler having a main absorption in the blue region of the spectrum, a colored cyan coupler having a main absorption in the green region of the spectrum, and a colorless cyan coupler, each coupler being capable of coupling with an oxidation product of a p-phenylenediamine color-developing agent to form a cyan dye and being present in a red-sensitive silver halide emulsion layer, said colored cyan coupler having a main absorption in the green region of the spectrum being a coupler represented by the following general formula (I)



(I)

wherein R<sub>1</sub> represents an aryl group; R<sub>2</sub> represents an aryl group having at least one of an alkoxy carbonyl group, an aryloxycarbonyl group, an alkyl carbonyl group or an aryl carbonyl group as a substituent; or the following general formula (II)



(II)

wherein R<sub>3</sub> represents an alkyl group; R<sub>4</sub> represents a monocyclic aryl group containing an alkoxy carbonyl group, an aryloxycarbonyl group, an alkyl carbonyl group or an aryl carbonyl group at the o-position with respect to the azo group; said colored cyan coupler having a main absorption in the blue region of the spectrum being a coupler represented by the following general formula (VII)



(VII)

wherein R<sub>12</sub> represents an alkyl group; and R<sub>13</sub> represents a monocyclic aryl group having an alkoxy carbonyl group or aryloxycarbonyl group at the m- or p-position with respect to the azo group; or the general formula (VIII)



(VIII)

wherein R<sub>14</sub> represents an alkyl group; R<sub>15</sub> represents an alkyl group or an aryl group; R<sub>16</sub> represents a monocyclic aryl group having at least one of an alkoxy carbonyl group or an aryloxycarbonyl group as a substituent; and said colorless cyan coupler being a coupler represented by the following general formula (XIV) or (XV)



(XIV)



(XV)

20 wherein R<sub>23</sub> and R<sub>24</sub> each represents a hydrogen atom, an alkyl group, a cyclic alkyl group, an aryl group, a heterocyclic group, or in combination the non-metallic atoms necessary for forming a heterocyclic ring; R<sub>27</sub> represents a hydrogen atom, an alkyl group, an aryl group, a heterocyclic group, an amino group, a carbonamido group, a sulfonamido group, a carbamyl group, or a ureido group; wherein R<sub>25</sub>, R<sub>26</sub>, R<sub>28</sub>, R<sub>29</sub> and R<sub>30</sub> each represents the groups as described with respect to R<sub>27</sub> and further represents a halogen atom or an alkoxy group; X and Y each represents a hydrogen atom, or a group capable of being eliminated on coupling with the oxidation product of an aromatic primary amine developing agent or X is a cyclic imido group or a residue capable of releasing a restrainer upon development.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410

wherein  $R_5$  represents a branched alkyl group having 6 to 22 carbon atoms; and  $R_6$  represents a lower alkyl group having 1 to 6 carbon atoms; the following general formula (IV)



wherein  $R_7$  represents a monocyclic aryl group having at least one alkoxy carbonyl group having 9 to 22 carbon atoms; and  $R_8$  represents a lower alkyl group having 1 to 6 carbon atoms; the following general formula (V)



wherein R<sub>9</sub> represents a naphthalene ring residue connected to the amido group of the  $\alpha$ -position thereof; and X represents an aryl group having at least one alkoxycarbonyl group containing 1 to 22 carbon atoms; or the general formula (VI)



wherein x represents an integer of 0 to 4; y represents 0 or 1; R<sub>10</sub> represents an aryl group or an alkyl group having 6 to 22 carbon atoms; and R<sub>11</sub> represents an alkyl group having 1 to 4 carbon atoms; and said colored cyan coupler having a main absorption in the blue region of the spectrum is a coupler represented by the following general formula (IX)



wherein  $R_{17}$  represents an alkyl group having 6 to 32 carbon atoms; and  $R_{18}$  represents an alkyl group having 1 to 20 carbon atoms; the following general formula (X)



20 wherein  $R_{17}$  and  $R_{18}$  are the same as defined above; the following general formula (XI)



wherein  $R_{17}$  and  $R_{18}$  are the same as defined above; the following general formula (XII)



60 wherein  $R_{19}$  and  $R_{20}$  each represents an alkyl group having 1 to 20 carbon atoms;  $R_{21}$  represents a monocyclic aryl group having at least one of an alkoxy carbonyl group or an aryloxy carbonyl group as a substituent; and  
65  $R_{22}$  represents an aryl group.

65  $R_{22}$  represents an aryl group.

6. The color photographic light-sensitive material of claim 1, wherein each of said couplers is incorporated in a different red-sensitive silver halide emulsion layer.

7. The color photographic light-sensitive material of claim 1, wherein two of said couplers are incorporated in the same red-sensitive silver halide emulsion layer and the third of said couplers is incorporated in a different red sensitive silver halide emulsion layer.

8. The color photographic light-sensitive material of claim 1, wherein all of said couplers are incorporated in the same red-sensitive silver halide emulsion layer.

9. The color photographic light-sensitive material of claim 1, wherein the amount of each of the colored cyan coupler having a main absorption in the blue region of the spectrum and of the colored cyan coupler having a main absorption in the green region of the

spectrum ranges from about 0.02 to about 2 moles per mol of the colorless cyan coupler; and wherein the molar ratio of silver to the colorless cyan coupler, the colored cyan coupler having a main absorption in the blue region of the spectrum and the colored cyan coupler having a main absorption in the green region of the spectrum ranges from about 4:1 to 100:1.

10. The color photographic light-sensitive material of claim 9, wherein the molar proportion of the colored cyan coupler having a main absorption in the blue region of the spectrum to the colored cyan coupler having a main absorption in the green region of the spectrum ranges from about 10:1 to 1:10.

\* \* \* \* \*

15

20

25

30

35

40

45

50

55

60

65